



US005944918A

**United States Patent** [19]**Keener**[11] **Patent Number:** **5,944,918**[45] **Date of Patent:** **Aug. 31, 1999**

[54] **METHOD FOR PREPARING PRE-COATED ALUMINUM ARTICLES AND ARTICLES PREPARED THEREBY**

[75] Inventor: **Steven G. Keener**, Trabuco Canyon, Calif.

[73] Assignee: **McDonnell Douglas Corporation**, Long Beach, Calif.

[21] Appl. No.: **08/726,792**

[22] Filed: **Oct. 7, 1996**

**Related U.S. Application Data**

[63] Continuation of application No. 08/432,223, May 1, 1995, Pat. No. 5,614,037.

[51] **Int. Cl.<sup>6</sup>** ..... **C23C 22/00**

[52] **U.S. Cl.** ..... **148/251; 148/264; 148/537; 148/688; 148/437; 148/439; 427/388.1**

[58] **Field of Search** ..... **148/537, 688-702, 148/251, 437, 439, 264; 427/388.1**

**References Cited****U.S. PATENT DOCUMENTS**

3,032,448 5/1962 Siebel et al. ..... 148/537  
3,065,108 11/1962 Seelig, et al. ..... 427/253

|           |         |                        |           |
|-----------|---------|------------------------|-----------|
| 3,123,516 | 3/1964  | Eiland .....           | 148/698   |
| 3,841,896 | 10/1974 | Boggs et al. .....     | 428/220   |
| 3,899,370 | 8/1975  | Takahashi et al. ..... | 148/518   |
| 3,983,304 | 9/1976  | Sekhon .....           | 411/504   |
| 4,115,607 | 9/1978  | Hasegawa .....         | 427/387   |
| 4,642,011 | 2/1987  | Uramoto et al. .....   | 411/258   |
| 5,077,096 | 12/1991 | Sharaby .....          | 427/388.2 |

**OTHER PUBLICATIONS**

SN 174078, May 11, 1943 (Alien Property Custodian).  
Anon "Material Safety Data Sheet for Hi-Kote 1", 2 pages (Feb. 9, 1994).  
Anon, "Material Safety Data Sheet for Alumazite ZY-138", 4 pages (Apr. 27, 1993).

*Primary Examiner*—David A. Simmons

*Assistant Examiner*—Robert R. Koehler

*Attorney, Agent, or Firm*—Alston & Bird LLP

[57]

**ABSTRACT**

An aluminum-alloy article such as a fastener is prepared by providing an aluminum-alloy article that is not in its final heat-treated state, and is preferably in its annealed state. A curable organic coating material is also provided. The method includes applying the organic coating material to the aluminum-alloy article, and heat-treating the coated aluminum article to its final heat-treated state, thereby simultaneously curing the organic coating.

**43 Claims, 2 Drawing Sheets**





**FIG. 1.**



**METHOD FOR PREPARING PRE-COATED  
ALUMINUM ARTICLES AND ARTICLES  
PREPARED THEREBY**

This is a continuation of application Ser. No. 08/432,223, filed May 1, 1995, now U.S. Pat. No. 5,614,037.

**BACKGROUND OF THE INVENTION**

This invention relates to the preparation of coated aluminum-alloy articles, and, more particularly, to the preparation of coated and heat-treated aluminum rivets.

Fasteners are used to mechanically join the various structural elements and subassemblies of aircraft. For example, a large transport aircraft typically includes over one million fasteners such as bolts, screws, and rivets. The fasteners are formed of strong alloys of metals such as titanium, steel, and aluminum alloys. In most cases, the fasteners are heat-treated, as by an aging treatment, to achieve as high a strength, in combination with other desirable properties, as is reasonably possible for that particular alloy. Heat-treating usually involves a sequence of one or more steps of controlled heating in a controlled atmosphere, maintenance at temperature for a period of time, and controlled cooling. These steps are selected for each particular material in order to achieve its desired physical and mechanical properties.

It has been the practice to coat some types of fasteners with organic coatings to protect the base metal of the fasteners against corrosion damage. In the usual approach, the fastener is first fabricated and then heat-treated to its required strength. After heat-treatment, the fastener is etched with a caustic soda bath to remove the scale produced in the heat-treatment. Optionally, the fastener is alodined or anodized. The coating material, dissolved in a volatile carrier liquid, is applied to the fastener by spraying, dipping, or the like. The carrier liquid is evaporated. The coated fastener is heated to elevated temperature for a period of time to cure the coating. The finished fastener is used in the fabrication of the structure.

This coating approach works well with fasteners made of a base metal having a high melting point, such as fasteners made of steel or titanium alloys. Such fasteners are heat-treated at temperatures well above the curing temperature of the coating. Consequently, the curing of the coating, conducted after heat-treating of the fastener is complete, does not adversely affect the properties of the already treated base metal.

On the other hand, aluminum alloys have a much lower melting point, and thence a generally much lower heat-treatment temperature, than steel and titanium alloys. It has not been the practice to coat high-strength aluminum-alloy fasteners with curable coatings, because it is observed that the curing treatment for the coating can adversely affect the strength of the fastener. The aluminum-alloy fasteners are therefore more susceptible to corrosion than would otherwise be the case. Additionally, the presence of the organic coating aids in the installation of the fastener for titanium alloys and steel. The absence of the coating means that aluminum fasteners such as rivets must be installed using a wet sealant compound for purposes of corrosion protection. The wet sealant compound is messy and difficult to work with, and may require extensive cleanup of the area around the fastener using caustic chemical solutions.

There exists a need for an improved approach to the protection of aluminum-based fasteners such as rivets. The present invention fulfills this need, and further provides related advantages.

**SUMMARY OF THE INVENTION**

The present invention provides a method for preparing an aluminum-alloy article such as a rivet. The article is heat-treated to high strength, and also is protected by a cured organic coating. The application of the coating does not adversely affect the properties of the article. The present approach is accomplished at an additional cost, of much less than one cent per fastener above its unprotected cost.

In accordance with the invention, a method for preparing an aluminum-alloy article comprises the steps of providing an aluminum-alloy article that is not in its final heat-treated state and providing a curable organic coating material. The coating material has a non-volatile portion that is predominantly organic and is curable at about a heat-treatment temperature of the aluminum-alloy article. The method further includes applying the organic coating material to the aluminum-alloy article by any suitable approach, and heat-treating the coated aluminum article to its final heat-treated state, thereby simultaneously curing the organic coating.

In the present approach, the article is preferably provided in an annealed or quenched condition suitable for the subsequent utilization of the strengthening heat-treatment, but not as yet heat-treated. The organic coating material, preferably dissolved in a suitable carrier liquid, is applied to the article which is not in its heat-treated state. The carrier liquid is removed by evaporation. The article is thereafter heat-treated to its full strength by heating to elevated temperature. During the heat-treatment according to the combination of temperature(s), time(s), and environment(s) specified for the aluminum-alloy base metal of the fastener, the coating is cured. Thus, no separate curing procedure is required after coating an already heat-treated article, which curing procedure would be likely to adversely affect the strength of the base metal of the article.

This approach yields surprising and unexpected technical and cost advantages when used in conjunction with high-strength aluminum fasteners such as rivets. The aluminum-alloy fasteners exhibit their full required strength produced by the heat-treatment used by itself. During installation, the fasteners need not be used in conjunction with wet sealants, wherein a viscous liquid sealant is applied to the fastener and faying surfaces just before upsetting the fastener. The elimination of the wet sealant installation approach for the over-700,000 rivets in a large cargo aircraft offers a cost savings of several million dollars per aircraft. The elimination of the use of wet sealants also improves the workmanship in the fastener installation, as there is no possibility of missing some of the fasteners as the wet sealant is applied. The coated fasteners are more resistant to corrosion during service than are uncoated fasteners.

Other features and advantages of the present invention will be apparent from the following more detailed description of the preferred embodiment, taken in conjunction with the accompanying drawings, which illustrate, by way of example, the principles of the invention.

**BRIEF DESCRIPTION OF THE DRAWINGS**

FIG. 1 is a process flow diagram for the method of the invention; and

FIG. 2 is a schematic sectional view of a protruding-head rivet fastener used to join two pieces, prior to upsetting;

FIG. 3 is a schematic sectional view of a slug rivet fastener used to join two pieces, prior to upsetting;

FIG. 4 is a schematic sectional view of a flush-head rivet fastener used to join two pieces, prior to upsetting; and

FIG. 5 is a schematic sectional view of the flush-head rivet fastener of FIG. 4, after upsetting.

#### DETAILED DESCRIPTION OF THE INVENTION

As depicted in FIG. 1, an untreated (i.e., uncoated and annealed) article is first provided. The preferred embodiment of the invention relates to the preparation of fasteners such as rivets, and the following discussion will emphasize such articles. The use of the invention is not limited to fasteners and rivets, and instead is more broadly applicable. However, its use in fasteners offers particular advantages that will be discussed.

A rivet 40 is provided, numeral 20. The present invention is used with a rivet, fastener, or other article manufactured to its conventional shape and size. FIGS. 2-4 illustrate three types of rivets 40, at an intermediate stage of their utilization to join a first piece 42 to a second piece 44, after installation to the first and second pieces but before upsetting. The rivet 40 of FIG. 2 has a premanufactured protruding head 46 on one end. The rivet 40' of FIG. 3, a slug rivet, has no preformed head on either end. The rivet 40" of FIG. 4 has a premanufactured flush head 46" on one end, that resides in a countersink in the piece 42.

The rivet 40 is manufactured of an aluminum-base alloy. As used herein, "aluminum-alloy" or "aluminum-base" means that the alloy has more than 50 weight percent aluminum but less than 100 weight percent aluminum. Typically, the aluminum-base alloy has about 85-98 weight percent of aluminum, with the balance alloying elements and a minor amount of impurity. Alloying elements are added in precisely controlled amounts to modify the properties of the aluminum alloy. Alloying elements that are added to aluminum in combination to modify its properties include, for example, magnesium, copper, and zinc, as well as other elements.

In the case of most interest, the aluminum alloy is heat-treatable. The alloying elements are selected such that the aluminum alloy can be processed to have a relatively soft state, as by annealing it at an elevated temperature for a period of time. The aluminum alloy in its soft state can be easily fabricated to form the rivet or other shape as shown in FIGS. 2-4. After the article is formed to its desired shape, it may be further processed to increase its strength several fold to have desired high-strength properties for service. The processing leading to strengthening is generally termed "heat-treating", wherein the article is subjected to one or more steps of exposure to an elevated temperature for a period of time, with heating and cooling rates selected to aid in producing the desired final properties. The temperatures, times, and other parameters required to achieve particular properties are known and are available in reference documents for standard aluminum-base alloys.

A specific aluminum-base alloy of most interest for rivet applications is an alloy which has a composition of about 2.3 weight percent copper, 2.2 weight percent magnesium, 6.2 weight percent zinc, 0.12 weight percent zirconium, balance aluminum plus minor impurities. (Other suitable alloys include, but are not limited to, 2000, 4000, 6000, and 7000 series heat-treatable aluminum alloys.) This alloy is available commercially from several aluminum companies, including ALCOA, Reynolds, and Kaiser. This alloy, designated 7050 alloy by the Aluminum Association, can be fully annealed (i.e., solution heat-treated) to have an ultimate shear strength of about 34,000-35,000 pounds per square inch (psi). (Aluminum Association terminology for alloy

types, heat-treatments, and the like are accepted throughout the art, and will be used herein.) In this state, the fastener is machined or otherwise formed into the desired shape of an article, in this case the rivet 40 such as shown in FIGS. 2-4. 5 This condition is termed the "untreated state" herein, as it precedes the heat-treatment required to increase the strength of the material. The article may be re-annealed after it is formed, prior to the strengthening heat-treatment.

After forming (and optionally re-annealing), the 7050 10 alloy may be heat-treated at a temperature of about 250° F. for 4-6 hours. The temperature is thereafter increased from 250° F. directly to about 355° F. for a period of 8-12 hours, followed by an ambient air cool. This state of heat-treatment, termed T73 condition, produces a strength of about 15 41,000-46,000 psi in the 7050 alloy, which is suitable for fastener applications.

A coating material is provided, numeral 22, preferably in 20 solution so that it may be readily and evenly applied. The usual function of the coating material is to protect the base metal to which it is applied from corrosion, including, for example, conventional environmental corrosion, galvanic corrosion, and stress corrosion. The coating material is a formulation that is primarily of an organic composition, but 25 which may contain additives to improve the properties. It is desirably initially dissolved in a carrier liquid so that it can be applied to a substrate. After application, the coating material is curable to effect structural changes within the organic component, typically cross linking of organic molecules to improve the adhesion and cohesion of the coating.

A wide variety of curable organic coating materials are 30 available. A typical and preferred coating material of this type has phenolic resin mixed with one or more plasticizers, other organic components such as polytetrafluoroethylene, and inorganic additives such as aluminum powder and/or strontium chromate. These coating components are 35 preferably dissolved in a suitable solvent present in an amount to produce a desired application consistency. For the coating material just discussed, the solvent is a mixture of ethanol, toluene, and methyl ethyl ketone. A typical sprayable coating solution has about 30 weight percent ethanol, about 7 weight percent toluene, and about 45 weight percent methyl ethyl ketone as the solvent; and about 2 weight percent strontium chromate, about 2 weight percent aluminum powder, balance phenolic resin and plasticizer as the coating material. A small amount of polytetrafluoroethylene may 40 optionally be added. Such a product is available commercially as "Hi-Kote 1" from Hi-Shear Corporation, Torrance, Calif. It has an elevated temperature curing treatment of 1-4 hours at 350-400° F., as recommended by the manufacturer.

The coating material is applied to the untreated fastener 45 article, numeral 24. Any suitable approach, such as dipping, spraying, or brushing, can be used. In the preferred approach, the solution of coating material dissolved in solvent is sprayed onto the untreated rivets. The solvent is removed from the as-applied coating by drying, either at ambient or slightly elevated temperature, so that the coated article is dry to the touch. The coated article is not suitable for service at this point, because the coating is not sufficiently adhered to the aluminum alloy base metal and because the coating is not sufficiently coherent to resist 50 mechanical damage in service.

In the case of the preferred Hi-Kote 1, the as-sprayed 55 coating was analyzed by EDS analysis. The heavier elements were present in the following amounts by weight: Al, 82.4 percent; Cr, 2.9 percent; Fe, 0.1 percent; Zn, 0.7 percent; and Sr, 13.9 percent. The lighter elements such as

carbon, oxygen, and hydrogen were detected in the coating but were not reported because the EDS analysis for such elements is not generally accurate.

The base metal of the rivet article and the applied coating are together heated to a suitable elevated temperature, numeral 26, to achieve two results simultaneously. In this single step, the aluminum alloy is heat-treated to its final desired strength state, and the coating is cured to its final desired bonded state. Preferably, the temperature and time treatment of step 26 is selected to be that required to achieve the desired properties of the aluminum alloy base metal, as provided in the industry-accepted and proven process standards for that particular aluminum-base alloy. This treatment may not produce the most optimal cure state for the coating, but it has been determined that the heat-treatment of the metal is less forgiving of slight variations from the optimal treatment than is the curing treatment of the organic coating. That is, the curing of the coating can sustain larger variations in time and temperature with acceptable results than can the heat-treatment of the metal. Thus, the use of the heat-treatment of the metal yields the optimal physical properties of the metal, and acceptable properties of the coating.

In the case of the preferred 7050 aluminum-base alloy and Hi-Kote 1 coating discussed above, the preferred heat-treating temperature is the T73 heat-treatment of 7050 alloy: 4–6 hours at 250° F., followed by a ramping up from 250° F. to 355° F. and maintaining the temperature at 355° F. for 8–12 hours, and an ambient air cool to ambient temperature.

Thus, the heat-treating procedure 26 involves longer times at temperature and higher temperatures than is recommended for the organic coating. There was initially a concern that the higher temperatures and longer times, beyond those required for curing the coating, would degrade the coating. This concern proved to be unfounded. The final coating 48, shown schematically in FIGS. 2–4, is strongly adherent to the base metal aluminum alloy and is also strongly internally coherent. (In FIGS. 2–4, the thickness of the coating 48 is exaggerated so that it is visible. In reality, the coating 48 is typically about 0.0003–0.0005 inches thick after treating in step 26.)

The coated and treated rivet 40 is ready for installation, numeral 28. The fastener is installed in the manner appropriate to its type. In the case of the rivet 40, the rivet is placed through aligned bores in the two pieces 42 and 44, as shown in FIG. 2. The protruding remote end 50 of the rivet 40 is upset (plastically deformed) so that the pieces 42 and 44 are captured between the premanufactured head 46 and a formed head 52 of the rivet. FIG. 5 illustrates the upset rivet 40" for the case of the flush head rivet of FIG. 4, and the general form of the upset rivets of the other types is similar. The coating 48 is retained on the rivet even after upsetting, as shown in FIG. 5.

The installation step reflects one of the advantages of the present invention. If the coating were not applied to the fastener, it would be necessary to place a viscous wet sealant material into the bores and onto the faying surfaces as the rivet was upset, to coat the surfaces. The wet sealant material is messy and difficult to work with, and necessitates extensive cleanup of tools and the exposed surfaces of the pieces 42 and 44 with caustic chemical solutions after installation of the rivet. Moreover, it has been observed that the presence of residual wet sealant inhibits the adhesion of later-applied paint over the rivet heads. The present coating approach overcomes both of these problems. Wet sealant is not needed or used during installation. The later-applied paint adheres well over the coated rivet heads.

The present invention has been reduced to practice with rivets made of 7050 alloy. The rivets, initially in the untreated state, were coated with Hi-Kote 1 and another coating material, Alumazite ZY-138. (Alumazite ZY-138 is a sprayable coating available from Tiodize Co., Huntington Beach, Calif. Its composition includes 2-butanone solvent, organic resin, and aluminum powder.) The coated rivets were heat-treated to T73 condition with the heat-treatment of 4–6 hours at 250° F., followed by a ramping up from 250° F. to 355° F. and maintaining the temperature at 355° F. for 8–12 hours, followed by an ambient air cool.

The coated rivets were mechanically tested in accordance with MIL-R-5674 to verify that they meet required ultimate double shear strength requirements of 41,000–46,000 pounds per square inch achieved by uncoated rivets. In the testing, the ultimate double shear strength was 42,500–43,500 pounds per square inch, within the permitted range. Cylindrical lengths of each type of coated rivet were upset to a diameter 1.6 times their initial diameter to evaluate driveability. No cracking or spalling of the coating was noticed on the periphery of the upset specimens. Rivets were also installed and subsequently removed to evaluate coating integrity using a scanning electron microscope. The coatings exhibited no signs of cracking, spalling, or any other unacceptable conditions or abnormalities. This latter result is particularly important and surprising. The coatings were retained on the rivets even after upsetting. Thus, the coatings remained in place to protect the rivet after installation, obviating any need for the use of wet sealants.

Although a particular embodiment of the invention has been described in detail for purposes of illustration, various modifications and enhancements may be made without departing from the spirit and scope of the invention. Accordingly, the invention is not to be limited except as by the appended claims.

What is claimed is:

1. A method for preparing an aluminum-alloy article comprising the steps of:  
providing an aluminum alloy article in an untreated state having a heat treatment temperature;  
providing a curable phenolic resin-containing organic coating curable at about the heat treatment temperature of the aluminum-alloy article;  
applying the phenolic resin-containing organic coating to the aluminum alloy article;  
heat-treating the phenolic resin-containing organic coated aluminum article to a final heat-treated state, thereby simultaneously curing the aluminum alloy article and the organic coating; and  
obtaining a coated aluminum alloy article having a shear strength greater than the article in the untreated state, said aluminum alloy article selected from the group consisting of 2000, 4000, 6000 and 7000 series aluminum alloys.
2. The method of claim 1, wherein the step of providing an aluminum-alloy article includes the step of providing an aluminum-alloy fastener.
3. The method of claim 1, wherein the step of providing an aluminum-alloy article includes the step of providing an aluminum-alloy article in its fully annealed state.
4. The method of claim 1, wherein the step of applying includes the step of spraying the organic coating material onto the aluminum-alloy article, and thereafter removing any volatile constituents from the sprayed coating.

5. The method of claim 1, wherein the step of heat-treating includes the step of aging the aluminum article.

6. The method of claim 1, wherein the step of providing an aluminum-alloy article includes the step of providing an article made of an alloy selected from the group consisting of 2000 series, 4000 series, 6000 series, and 7000 series aluminum alloys.

7. The method of claim 1, including an additional step, after the step of heat-treating, of fastening a first piece to a second piece using the heat-treated article.

8. The method of claim 7, wherein the step of fastening includes the step of completing the fastening without using any wet sealant between the article and the pieces.

9. An article prepared by the method of claim 1.

10. A fastener prepared according to the method of claim 1.

11. The method according to claim 1, wherein the coating material is provided in solution.

12. The method according to claim 1, wherein the coating material is dissolved in a carrier.

13. The method according to claim 1, wherein the coating material comprises a phenolic resin and an organic solvent.

14. The method according to claim 1, wherein the coating material for comprises a plasticizer.

15. The method according to claim 1, wherein the coating material comprises polytetrafluoroethylene.

16. The method according to claim 1, wherein the coating material further comprises an inorganic compound selected from the group consisting of aluminum powder and strontium chromate.

17. A method for preparing an aluminum-alloy fastener, comprising the steps of:

providing an aluminum-alloy fastener in an untreated state;

providing a corrosion-resistant, phenolic resin-containing curable organic coating material, the coating having a non-volatile portion that is predominantly organic;

applying the phenolic resin-containing organic coating material to the aluminum-alloy fastener article;

heating the coated aluminum-alloy fastener to a temperature sufficient to simultaneously heat-treat the aluminum-alloy fastener and cure the organic coating; and

obtaining a coated aluminum-alloy fastener having a shear strength approximately equal to or greater than 34,000 psi.

18. The method of claim 17, wherein the step of applying includes the step of

spraying the organic coating material onto the aluminum-alloy article, and thereafter

removing any volatile constituents from the sprayed coating.

19. The method of claim 17, wherein the step of providing an aluminum-alloy article includes the step of

providing an article made of an alloy selected from the group consisting of 2000 series, 4000 series, 6000 series, and 7000 series aluminum alloys.

20. The method of claim 17, including an additional step, after the step of heat-treating, of

fastening a first piece to a second piece using the heat-treated article.

21. The method of claim 20, wherein the step of fastening includes the step of

completing the fastening without using any wet sealant between the article and the pieces.

22. An article prepared by the method of claim 17.

23. An article prepared according to the method of claim 17.

24. An article prepared by a method comprising the steps of

providing a rivet made from a 7050 aluminum-alloy in an untreated state;

providing phenolic resin-containing organic coating material;

applying the organic coating material to the aluminum-alloy rivet; and

heating the coated rivet to a temperature of from about 250° F. for a first period of time, and thereafter increasing the temperature to about 355° F. for a second period of time, to heat-treat the aluminum-alloy and cure the organic coating to achieve a coated rivet having a shear strength of approximately equal to or greater than 34,000 psi.

25. A method of making an aircraft comprising the steps of:

providing aircraft subassemblies;

providing aluminum-alloy articles in an untreated state;

providing a phenolic resin-containing curable organic coating material curable at about a heat treatment temperature of the aluminum-alloy fastener articles; coating the fastener articles with the coating material; heat treating the coated articles to a temperature sufficient to both heat-treat the aluminum-alloy articles and cure the organic coating;

cooling the coated articles to about room temperature such that the coated articles have a shear strength approximately equal to or greater than 34,000 psi.; and fastening the subassemblies together with the coated articles.

26. The method according to claim 25, wherein the aluminum-alloy fastener articles comprise 2000, 4000, 6000 and 7000 series heat-treatable aluminum alloys.

27. The method according to claim 25, wherein the fastener articles have an ultimate shear strength of from about 34,000 to about 35,000 psi.

28. The method according to claim 25, wherein the step of the coated fastener articles heating comprises first heat-treating the fastener articles at a temperature of from about 250 degrees F. for about 4 to about 5 hours, followed by a second heat-treatment of about 355 degrees F. for about 8 to about 12 hours.

29. The method according to claim 25, wherein the fastener articles have a strength of from about 41,000 to about 46,000 psi.

30. The method according to claim 25, wherein the fastener articles are selected from the group consisting of bolts, screws and rivets.

31. The method according to claim 25, wherein the fastener articles comprise rivets.

32. An aircraft made according to the method of claim 25.

33. An aircraft comprising aluminum-alloy fasteners, the fasteners coated with a phenolic resin-containing curable organic coating and heat-treated at a preselected temperature sufficient to both heat-treat the aluminum-alloy fasteners and cure the organic coating, said treated fasteners having a shear strength greater than the article in the untreated state, said aluminum alloy selected from the group consisting of 2000, 4000, 6000 and 7000 series aluminum alloys.

- 34.** The aircraft according to claim **33**, wherein the coating material is provided in solution.
- 35.** The aircraft according to claim **33**, wherein the coating material is dissolved in a carrier.
- 36.** The aircraft according to claim **33**, wherein the <sup>5</sup> coating material comprises a phenolic resin and an organic solvent.
- 37.** The aircraft according to claim **33**, wherein the coating material comprises a plasticizer.
- 38.** The aircraft according to claim **33**, wherein the <sup>10</sup> coating material comprises polytetrafluoroethylene.
- 39.** The aircraft according to claim **33**, wherein the coating material further comprises an inorganic compound selected from the group consisting of aluminum powder and strontium chromate.
- 40.** The aircraft according to claim **33**, wherein the <sup>15</sup> aluminum-alloy fasteners comprise 2000, 4000, 6000 and 7000 series heat-treatable aluminum-alloys.
- 41.** The aircraft according to claim **33**, wherein the coated aluminum-alloy heating step comprises first heat-treating <sup>20</sup> the fastener articles at a temperature of from about 250 degrees F. for about 4 to about 5 hours, followed by a second heat-treatment of about 355 degrees F. for about 8 to about 12 hours.

- 42.** The aircraft according to claim **41**, wherein the heat-treatments produce an alloy having a strength of from about 41,000 to about 46,000 psi.
- 43.** A method for preparing an aluminum-alloy article comprising the steps of:
- providing an aluminum-alloy article in an untreated state
- having a heat-treatment temperature;
- providing a phenolic resin-containing curable organic coating material curable at about the heat-treatment temperature of the aluminum-alloy article;
- applying the organic coating material to the aluminum-alloy article; and
- heat-treating the coated aluminum-article to the final heat-treated state, thereby simultaneously curing the organic coatings and obtaining a coated aluminum-alloy article having a shear strength greater than the article in the untreated state, said aluminum alloy selected from the group consisting of 2000, 4000 6000 and 7000 series aluminum alloys.

\* \* \* \* \*

UNITED STATES PATENT AND TRADEMARK OFFICE  
CERTIFICATE OF CORRECTION

PATENT NO. : 5,944,918

DATED : August 31, 1999

INVENTOR(S) : Keener

It is certified that error appears in the above-identified patent and that said Letters Patent is hereby corrected as shown below:

On the title page, [56] References Cited, OTHER PUBLICATIONS, line 1, before "Alien" insert --Dürr--; after "Custodian" insert --Report--; line 2, after "Anon" insert a comma (,).

Column 6, line 39, "at" should read --an--.

Column 7, line 27, cancel "for"; lines 47-48, indent sub-paragraph.

Column 8, line 3, "claim 17" should read --claim 1--; line 36, after "psi" cancel the period (.); lines<sup>45-46</sup>, claim 28, "step of the coated fastener articles heating" should read --heating step of the coated fastener articles--.

Column 10, line 16 "aluminum-article" should read --aluminum-alloy article--; line<sup>18</sup>, "coatings" should read --coating--.

Signed and Sealed this  
Twenty-ninth Day of February, 2000

Attest:



Q. TODD DICKINSON

Attesting Officer

Commissioner of Patents and Trademarks